

1

2,981,589

## CELLULOSE TREATMENT AND PRODUCT

Walter L. Hochner, Wilmington, Del., and Abb L. Scarbrough, Rahway, N.J., assignors to National Lead Company, New York, N.Y., a corporation of New Jersey

No Drawing. Filed May 21, 1958, Ser. No. 736,680

7 Claims. (Cl. 8—116.2)

This invention relates to a novel method for the treatment of fibrous cellulosic materials. In particular, this invention relates to a method for the treatment of fibrous cellulosic materials to render them hydrophobic and to impart water repellancy to articles made therefrom.

Many types of agents have been proposed for the treatment of fibrous materials to make them water-repellant. In general, these have consisted for the most part of various impregnating techniques whereby water-repelling agents, such as oils, waxes, synthetic resins or similar agents were deposited on the fiber and in the interstices between fibers, either to seal up the pores and thus prevent passage of water therethrough, or to impart a hydrophobic character to the surface, thus retarding the passage of moisture by the utilization of surface-tension effects.

These methods, however, suffered from certain disadvantages. The type of treatment which depended on a sealing of the pores was undesirable for many purposes because it made the fabric impervious to passage of air as well, so that the fabric was unable to "breathe." Treatments which depended on the imparting of a hydrophobic surface to the fiber overcame this disadvantage, but consisted primarily of impregnations or deposits of synthetic resins which were soluble in organic solvents and hence not capable of withstanding dry-cleaning.

An object of this invention, therefore, is to provide an improved process for treatment of fibrous cellulosic materials. Another object is to provide an improved process for imparting hydrophobic characteristics to fibrous cellulosic materials. A further object is to provide a method for imparting water-repellancy to cellulosic fabrics. A still further object is to impart, to a cellulosic fabric, water-repellant properties which are not removed by dry-cleaning. Other objects and advantages will become apparent from the following more complete description and claims.

Broadly, this invention contemplates a method for the treatment of a fibrous cellulosic material, which comprises the steps of partially carboxyalkylating a cellulosic material to extent that between one-third and one-fifteenth of the hydroxymethyl groups originally present in said cellulosic material are converted to carboxyalkoxymethyl groups and treating said partially carboxyalkylated cellulose with a quaternary ammonium halide having at least one alkyl group containing at least 12 carbon atoms.

This invention also contemplates, as a new article of manufacture, a modified cellulosic material characterized in that between one-third and one-fifteenth of the original anhydroglucose units of said cellulose are representable by the formula



wherein R represents a divalent alkyl hydrocarbon radical containing from 1 to 5 carbon atoms, and the four

2

R' groups are monovalent alkyl hydrocarbon radicals which may be the same or different, each R' group containing from 1 to 18 carbon atoms, at least one of said R' groups containing at least 12 carbon atoms.

5 The carboxyalkylation of the cellulose must be partial, and within the range above specified. If more than about  $\frac{1}{3}$  of the hydroxymethyl groups of the original cellulose structure are carboxyalkylated, the cellulose itself becomes water-soluble, or at least colloidally water-dispersable, and is unsuited to the production of a hydrophobic modified cellulosic material. If, on the other hand, less than about  $\frac{1}{15}$  of the original hydroxymethyl groups are carboxyalkylated, there are not enough carboxyalkyl groups in the molecule to react with the necessary quantity of amine salt, and the degree of water-repellancy will be impaired.

10 The carboxyalkylation of the hydroxymethyl groups is essential. It has been attempted to introduce the amine group into the cellulose molecule in a slightly different fashion, by oxidizing the hydroxymethyl group with  $\text{NO}_2$ , thereby converting it to a carboxyl group, and then forming the amine salt of that carboxyl group. This procedure produces a measurable, but much impaired and unsatisfactory degree of water-repellancy.

15 25 The reason for this difference in reactivity between a simple  $-\text{COOH}$  group and a  $-\text{CH}_2\text{O}-\text{R}-\text{COOH}$  group according to the invention is not fully established, but is believed to be a result of steric effects.

20 30 The term "carboxyalkoxymethyl," as used herein to describe the group resulting from modification of the hydroxymethyl group of the original cellulose molecule, is employed for the sake of simplicity, and is intended to embrace both the carboxyalkoxymethyl group itself,  $-\text{CH}_2\text{O}-\text{R}-\text{COOH}$ , and its alkali salts, e.g.



35 40 The carboxyalkylation of the cellulose molecule is accomplished in known manner, i.e. by treating the cellulose with a halogen-substituted alkanoic acid such as chloroacetic acid, dichloroacetic acid, chloropropionic acid or the like, in an aqueous alkaline solution such as a solution of sodium hydroxide. Any halogen-substituted alkanoic acid containing up to about 5 carbon atoms may be employed, but it is preferable, primarily for economic reasons, to employ short-chain, singly-substituted acids such as monochloroacetic acid. Similarly, any alkali may be employed but there is no advantage in using the relatively expensive potassium hydroxide or the other even more expensive alkalis, sodium hydroxide being quite adequate for the purpose. Alkaline earths, such as  $\text{Ba}(\text{OH})_2$ ,  $\text{Ca}(\text{OH})_2$ , etc. are, however, insufficiently alkaline.

45 50 55 The degree of carboxyalkylation of the cellulose is controlled by the reaction conditions, particularly the concentrations of acid and alkali and the time and temperature at which the reaction is carried out. It has been found that with a solution of 2% sodium hydroxide and 2% monochloroacetic acid in water, approximately  $\frac{1}{8}$  of the hydroxymethyl groups are carboxyalkylated in 15 minutes at  $50^\circ\text{C}$ . These reaction conditions are illustrative and obviously may be varied, as will be obvious to those skilled in the art. Thus, the concentration of alkali may be as low as about 1% or as high as about 10%. The higher concentrations of alkali favor more rapid and complete reaction, and also favor a partial mercerization, involving other hydroxymethyl groups than those which are carboxyalkylated. The mercerization effect takes place as a side reaction which is ordinarily not an undesirable one.

60 65 70 Similarly, the concentration of the acid may vary between about 1 and about 10%, the higher concentra-

tions favoring more complete and rapid carboxyalkylation.

The temperature and the time are mutually interdependent to some extent; thus, with conditions otherwise the same, the desired degree of carboxyalkylation can be achieved by a few minutes' treatment at temperatures above 50° C. and up to about 100° C., or by a protracted treatment for several hours at room temperature (say 25° C.), or slightly higher. At the higher temperatures, the progress of the reaction is, naturally, more difficult to control precisely, while at the lower temperatures, treatment times tend to be unduly extended, and it has been found most convenient to operate at intermediate temperatures.

The cellulosic material employed according to this invention may be in its natural state or may have undergone a previous modification according to known methods. For example, the original cellulose may have been partially acetylated, or partially nitrated, or converted to viscose or cuprammonium rayon, etc. It is essential, however, that at least  $\frac{1}{15}$  of the original  $-\text{CH}_2\text{OH}$  groups be present, either unmodified or regenerated. In this connection, it should be noted that the degree of carboxyalkylation specified above, viz. from  $\frac{1}{3}$  to  $\frac{1}{15}$  of the hydroxymethyl groups, is based on the hydroxymethyl groups originally present in the cellulose molecule, not of those remaining after any such prior treatment.

When the cellulose has been partially carboxyalkylated as just described, the resulting carboxyalkyl groups are converted to quaternary amine salts by metathetical exchange with a suitable quaternary amine halide. As noted above, the carboxyalkyl group may be in the alkali salt form, e.g.  $-\text{R}-\text{COONa}$ , in which case the alkali metal ion is replaced by the quaternary ammonium cation, forming an alkali halide by-product. Where the carboxyalkyl group is present in the acid form, i.e.  $-\text{R}-\text{COOH}$ , the reaction is the same, except that the by-product is a hydrohalic acid.

The quaternary ammonium salt is of the form



where the  $\text{R}'$  groups are monovalent alkyl hydrocarbon radicals containing from 1 to 18 carbon atoms, and may be the same or different and  $\text{X}$  is an ionizable anion, preferably a halide ion. Among the  $\text{R}'$  groups, it is essential that at least one of them be a long-chain radical having at least 12 carbon atoms; otherwise, the modified cellulosic material does not have the desired hydrophobic properties. Preferably, at least two of the  $\text{R}'$  groups should be long-chain radicals and preferably, the chains should be about 16 to 18 carbon atoms in length, rather than the minimum of 12. Suitable quaternary ammonium salts therefore include, as a few random examples, dodecyl trimethyl ammonium chloride, tetradecyl triethylammonium bromide, hexadecyl triisopropylammonium iodide, octadecyl tributylammonium sulfate, etc. Particularly preferred quaternary ammonium salts, containing at least two long-chain radicals, include didodecyl dimethylammonium chloride, ditetradecyl diethylammonium bromide, dihexadecyl diisopropylammonium iodide, dioctadecyl dimethylammonium chloride, tridodecyl monomethylammonium chloride, tritetradecyl monoethylammonium bromide, trihexadecyl monoisopropylammonium iodide, trioctadecyl monomethylammonium chloride, tetradodecylammonium chloride, tetrahexadecylammonium bromide, tetraoctadecylammonium chloride, tetracontylammonium sulfate, etc.

The reaction between the quaternary ammonium salt and the partially carboxyalkylated cellulosic material proceeds without difficulty and may be carried out at any convenient temperature between room temperature and the boiling point of the solvent (ordinarily water). The reaction is rapid and is complete within a few min-

utes, even at room temperature. Although this reaction may be carried out as a separate step, completely apart from the carboxyalkylation step, it is more convenient, and for reasons which are not known, also more effective to carry out the two reactions simultaneously, by dissolving the quaternary ammonium salt in the same solution of acid and alkali that is used to effect the carboxyalkylation. Thus, instead of using a solution of 2% NaOH and 2% monochloroacetic acid to carboxymethylate, as described above, and subsequently using a separate solution of a quaternary ammonium halide to convert the carboxymethyl group to its quaternary ammonium salt, it has been found effective to employ a solution containing 2% NaOH, 2% monochloroacetic acid and 2% dioctadecyl dimethylammonium chloride, and perform both steps in a single operation. The reaction conditions are not affected by the presence of the quaternary ammonium salt and, as above, may suitably consist of a 15 minute treatment at 50° C. Also, the concentration of the quaternary ammonium salt in the solution is not critical; it is limited only by solubility on the one hand and the necessity of having sufficient ammonium salt to react with the carboxyalkyl groups on the other.

In order to illustrate more fully the nature of this invention, the following examples are presented:

#### Example I

A treating solution was prepared by dissolving 2 kg. of NaOH, 2 kg. of monochloroacetic acid, and 2 kg. of dioctadecyl dimethylammonium iodide in water, and diluting the solution to a volume of 100:1. The solution was heated to 50° C. A sample of cotton twill, weighing 8.2 oz. per square yard, was steeped in the heated solution for 15 minutes, then withdrawn, washed with water, and dried. The dried cloth was then subjected to a water-repellancy test as described in the Technical Manual and Year Book of the American Association of Textile Chemists and Colorists, volume 27, 1951, Resistance to Wetting, Standard Test Method 22-41, page 133.

The treated cotton twill tested in this manner obtained a rating of 70. By comparison, an untreated sample of the same cloth was also subjected to the same test and was completely wetted with a rating of zero.

The treated material was laundered several times and subjected, after each laundering, to the same above mentioned wetting test. It was found that the treated material maintained its rating of 70 after each laundering.

#### Example II

A sample of cotton twill, weighing 8.2 oz. per square yard was placed in a 15% solution of monochloroacetic acid for two minutes. The excess acid was then squeezed out, and the cotton twill placed in a 50% sodium hydroxide solution at 80° C. for 60 seconds. The cloth was then removed from the solution, and the excess hydroxide was removed by continuous washing with water.

The degree of carboxyalkylation was determined by taking a dry, weighed sample of this treated cloth, and dissolving the free acid therein in a known excess of standard base, and titrating the excess base with phenolphthalein. The degree of carboxyalkylation was thus determined to be  $\frac{1}{15}$  of the hydroxymethyl groups originally present.

The remainder of the treated cloth was then immersed in a 2% solution of dodecyl trimethylammonium chloride for 15 minutes at 50° C. The cloth was then rinsed with water and dried.

The water repellancy test of Example I was then repeated using the treated cloth of this Example II. The treated cloth of the present example obtained a rating of 60. The treated material of this example was subjected to several launderings and after each laundering, the water repellancy test was repeated. It was found that

the treated material of this example maintained its rating of 60.

*Example III*

The procedure of Example II was repeated, but the cotton twill was placed in a 30% monochloroacetic acid solution for six minutes, the excess acid squeezed out, and the cotton twill was then placed in a 50% sodium hydroxide solution at 80° C. for two minutes.

The degree of carboxyalkylation was determined as in Example II, and was ascertained to be  $\frac{1}{3}$  of the hydroxymethyl groups originally present.

The remainder of the treated cloth was then subjected to the same procedure as in Example II, except that the tetradecyl triethylammonium bromide was used in place of the dodecyl trimethylammonium chloride used in Example II.

The water repellency test of Example I was then repeated using the treated cloth of this Example III.

The treated cloth of the present example obtained a rating of 80. The treated material of this example was subjected to several launderings and after each laundering, the water repellency test was repeated. It was found that the treated material of this example maintained its rating of 80.

*Example IV*

The procedure of Example I was repeated, except that an equivalent amount of omega monochloropentanoic acid was used in place of the monochloroacetic acid used in Example I.

The treated cotton twill was subjected to the same tests as in Example I. A rating of 70 was obtained both before and after laundering.

The process of this invention is simple and economical. It is effective to provide, in cellulosic materials, hydrophobic properties and water-repellency which are not subject to removal by exposure to organic solvents. It is applicable to cellulosic materials in general, including fabrics such as cotton, linen, regenerated cellulose, viscose and cellulose acetate, also natural fibers such as kapok, hemp, wood and wood products such as pressed board, cardboard, batting, paper, wood flour, sawdust and the like.

The modified cellulose according to this invention is a new article of commerce possessing unique properties, outstanding among which are the combination of a cellulosic structure with a hydrophobic character which is not susceptible of removal by exposure to organic solvents.

While this invention has been described with reference to certain specific embodiments and illustrated by certain examples, these are illustrative only, and the invention is not to be construed as limited, except as set forth in the appended claims.

We claim:

1. A method for the treatment of a fibrous cellulosic textile material, at least one-fifteenth of the hydroxymethyl groups originally present in said material being present in unsubstituted form, which comprises the steps of partially carboxyalkylating said cellulosic material under non-dissolving conditions, to maintain the fibrous form, to the extent that between one-third and one-fifteenth of the hydroxymethyl groups originally present in said cellulosic material are converted to carboxyalkoxymethyl groups and treating said non-dissolved, partially carboxyalkylated cellulose with a quaternary ammonium halide having at least one alkyl group containing from 12 to 18 carbon atoms.
- 15 2. A method according to claim 1, wherein said quaternary ammonium halide is dodecyl trimethylammonium chloride.
- 20 3. A method according to claim 1, wherein said quaternary ammonium halide is tetradecyl triethylammonium bromide.
- 25 4. A method according to claim 1, wherein said quaternary ammonium halide is dioctadecyl dimethylammonium iodide.
5. As a new article of manufacture, a modified cellulosic textile material characterized in that between one-third and one-fifteenth of the original anhydro-glucose units of said cellulose are representable by the formula

30



wherein R represents a divalent alkyl hydrocarbon radical containing from 1 to 5 carbon atoms and the four R' groups are monovalent alkyl hydrocarbon radicals which may be the same or different, each R' group containing from 1 to 18 carbon atoms, at least one of said R' groups containing at least 12 carbon atoms.

35 6. As a new article of manufacture according to claim 5, a water repellent cellulosic fabric.

7. As a new article of manufacture according to claim 5, a modified cellulosic material, wherein the modified anhydroglucose units are stable in the presence of organic solvents and of water.

45

References Cited in the file of this patent

UNITED STATES PATENTS

|              |                  |               |
|--------------|------------------|---------------|
| 50 2,313,741 | Engelmann et al. | Mar. 16, 1943 |
| 2,314,277    | Hurd             | Mar. 16, 1943 |
| 2,448,153    | Reid et al.      | Aug. 31, 1948 |
| 2,681,846    | Guthrie et al.   | June 22, 1954 |
| 2,729,535    | Balassa et al.   | Jan. 3, 1956  |
| 2,840,446    | Compton et al.   | June 24, 1958 |